

Aug. 30, 1927.

F. SKAUPY ET AL

1,640,428

ELECTRODE FOR ELECTRIC DISCHARGE DEVICES

Filed Oct. 30, 1923



Inventors:  
Franz Skaupy,  
Marcello Pirani,  
Fritz Bahr,  
Werner Fehse,

by *Alexander S. Lint*  
Their Attorney.

## UNITED STATES PATENT OFFICE.

FRANZ SKAUPY, MARCELLO PIRANI, FRITZ BAHR, AND WERNER FEHSE, OF BERLIN,  
GERMANY, ASSIGNORS TO GENERAL ELECTRIC COMPANY, A CORPORATION OF  
NEW YORK.

## ELECTRODE FOR ELECTRIC-DISCHARGE DEVICES.

Application filed October 30, 1923, Serial No. 671,795, and in Germany December 22, 1922.

The present invention relates to the manufacture and construction of non-consuming electrodes of concentrated mass for electric arc lamps or similar electric discharge devices.

Heretofore tungsten electrodes of concentrated mass, such as used for example in lamps or similar devices in which an arc is operated in a gas, have been made by fusing the lower end of a piece of tungsten wire held in a vertical position until a spherical molten drop of tungsten is formed at the heated end of the wire. Since a heavy drop of tungsten easily breaks off it has been possible to obtain by this process with stem wires of suitable size only comparatively small spherical electrodes, say about 3.5 to 4 m. m. in diameter. The spherical electrode bodies often have hollow spaces in the interior which are formed at the high temperature of fusion by the evaporation of small amounts of impurities present in even the best purified tungsten. The hollow spaces in the electrodes are harmful as they tend to produce inequalities of temperature in the electrode bodies and decrease the length of life of the arc electrode.

According to the process constituting the present invention, electrodes of refractory metal of which tungsten is an example, are made from powdered metal which first is partially consolidated by compression and preliminary sintering, then is joined to a supporting stem and is finally further consolidated by heating to high incandescence in an inert environment. The shrinking of the electrode body upon the stem according to this process produces a most intimate and firm connection between the stem and the body. The resulting electrodes are dense and free from cavities.

A more complete understanding of our invention may be had from the following description taken in connection with the accompanying drawing in which Fig. 1 represents an illustrative form of electrode, and Fig. 2 illustrates in vertical section a suitable furnace for carrying out our invention.

In the production of electrode bodies the finely divided metal is shaped by pressing in a suitable mold (not shown) to a desired

form, preferably somewhat larger than the dimensions desired in the finished article. It is not necessary in our process to adhere to a spherical shape, in fact it is advantageous to produce hemispherical electrode bodies having a flat surface, as shown in Fig. 1. An electrode of this shape has the advantage that when lamps containing the same are used in projectors for motion pictures or the like, the total light radiation is concentrated on the film to be projected. The pressed electrodes are next given a preliminary sintering operation by heating to a temperature sufficiently high to partially consolidate the metal, (say, a temperature of 1300°). This firing treatment renders the bodies sufficiently hard to be worked mechanically. If desired, the shape of the electrodes may be changed by mechanical means and the smoothness of the surface improved. At this stage of manufacture a hole is mechanically made in the electrodes, as by boring and a supporting stem, also consisting of tungsten, molybdenum, or other refractory material, preferably of wrought metal, is inserted loosely in the depression in the electrode body before the final sintering.

The stem of the electrode may to advantage be inserted obliquely as shown in the drawing. This shape of electrode prevents creeping up of the arc from the electrode itself to the supporting stem. The final step in the manufacture of the electrodes consists in sintering at bright incandescence (to a temperature of about 3000°), in order to completely consolidate the electrode mass 1, and to shrink the same upon the relatively thin inserted stem 2. Although this final step may be carried out in any suitable device, it may to advantage be carried out in a tube furnace, as shown in Fig. 2 of the drawing. This furnace as diagrammatically indicated comprises a cylindrical tank *a*, which is closed at the lower end by a mercury packing *b*, contained within a channel in a plate *p*. The two water cooled current supply conductors *c*, *d*, project through the base plate *p* into the interior. The current conductor *c* is connected to a small tank *e* containing mercury, in the interior of which is mounted a cool-

ing coil *f*. Into this body of mercury projects a terminal *g* of a tube *h*, preferably consisting of tungsten.

The terminal *g* conveniently is constituted of hinged jaws held in firm relation to the tube *h* by a spring *s*. The tube *h* is held at the opposite end by a clamp terminal *i*, attached to the current supply conductor *d*. The partially sintered electrode bodies *k* provided as above described with inserted stems, are placed within the heater tube *h*, the lower end of which is closed in any suitable manner, as for example, by means of a wad of tungsten wire. The tank *a* during the sintering operation is supplied with hydrogen, which enters by a tube *m* and leaves the tank through a tube *n*. The tungsten tube *h* is heated to incandescence by the passage of current. The inserted electrodes *k* are sintered by radiated heat and become firmly united with the supporting stems. After the completion of the sintering process the electrodes may be directly mounted in lamps or other electric discharge devices.

One of the advantages of the present process is the homogeneity and freedom from cavities of the electrodes made thereby, and furthermore, the electrodes may be given any desired size and form in pressing.

What we claim as new and desire to secure by Letters Patent of the United States, is:

1. The method of making electrodes of refractory metal which consists in compressing powdered refractory metal to desired form, sintering to partially consolidate the same, inserting a stem and completing the consolidation by sintering at a higher temperature. 35

2. The method of making electrodes of tungsten which consists in pressing powdered tungsten to desired form, partially consolidating at an elevated temperature, inserting a stem and completing the consolidation by heating the article to a higher temperature below the fusion temperature of tungsten. 45

3. An electrode comprising a mass of sintered refractory metal having a flat surface and a relatively thin stem of wrought metal oblique to said surface and imbedded in and united with said sintered mass. 50

In witness whereof, we have hereunto set our hands this 8th day of October, 1923.

FRANZ SKAUPY.  
MARCELLO PIRANI.  
FRITZ BAHR.  
WERNER FEHSE.